

No. 747,282.

PATENTED DEC. 15, 1903.

B. WALLGREN.

FIRE KINDLER.

APPLICATION FILED JULY 15, 1903.

NO MODEL.



Witnesses  
E. H. Stewart  
C. N. Woodward.

Bengt Wallgren, Inventor  
by *C. H. Snow & Co.*  
Attorneys

## UNITED STATES PATENT OFFICE.

BENGT WALLGREN, OF EAST RUTHERFORD, NEW JERSEY, ASSIGNOR OF  
TWO-THIRDS TO ARTHUR C. VAN RODEN AND GARRET VAN WAG-  
ONER, OF EAST RUTHERFORD, NEW JERSEY.

## FIRE-KINDLER.

SPECIFICATION forming part of Letters Patent No. 747,282, dated December 15, 1903.

Application filed July 15, 1903. Serial No. 165,592. (No model.)

*To all whom it may concern:*

Be it known that I, BENGT WALLGREN, a citizen of the United States, residing at East Rutherford, in the county of Bergen and State 5 of New Jersey, have invented a new and useful Fire-Kindler, of which the following is a specification.

This invention relates to fire-kindlers of the class composed of compounds of inflammable 10 or combustible materials, and has for its object to simplify and improve articles or products of this character; and it consists in combining rosin, tallow, and woody material in the manner and in about the proportions herein- 15 after described.

In producing the improved article rosin and tallow are melted and combined and applied as a coating to a relatively thin slab of wood or woody material and an outer coating of 20 wood-shavings, excelsior, wood-pulps, or the like added to the rosin and tallow compound before they harden.

For the purpose of illustrating the manner of producing the improved fire-kindler a perspective figure is shown in the drawing representing the various steps employed in its 25 production.

In the illustration, 10 represents the foundation or base, which may be of soft wood or 30 other woody material, 11 the coating of combined rosin and tallow, and 12 the outer layer of shavings, excelsior, paper-pulp, or similar material, preferably in finely-divided particles, as shown.

35 The foundation member 10 governs the size and configuration of the product, and this will preferably be relatively thin and of material which is at the same time cheap and readily combustible and which will impart

sufficient heat and flame to ignite the surrounding fuel, especially relatively refractory material, such as anthracite coal. By this means a fire-kindler is produced which may be cheaply manufactured, easily applied, and which will not be dangerous either in operation or from a tendency to ignite spontaneously or at a low temperature. The "bricks" or "slabs" thus formed may be stored, therefore, with as great safety as ordinary soft-wood kindlings. A brick or slab thus constructed may be embedded in the fuel to be ignited and when fire is applied will burn fiercely and in turn ignite the contiguous and surrounding fuel, as will be obvious.

In the manufacture of the article I employ 55 a compound formed of ten parts of rosin to eight parts of tallow, by weight, and these are thoroughly mixed together and then applied as a coating to the wood.

Having thus described the invention, what 60 I claim is—

As a new article of manufacture, a fire-kindler composed of a foundation or core of wood, an inner coating or envelop of rosin and tallow combined in the proportions of 65 eight parts of tallow and ten parts of rosin, and an outer envelop of finely-divided woody material such as shavings, wood-pulp or the like loosely arranged upon the coating of rosin and tallow.

70 In testimony that I claim the foregoing as my own I have hereto affixed my signature in the presence of two witnesses.

BENGT WALLGREN.

Witnesses:

CHARLES LINDSTROM,  
MARIAN E. NIEDERER.